

June 9, 1953

J. J. DUNN ET AL  
METHOD AND MEANS FOR INCREASING BENDING FATIGUE  
STRENGTH OF ROTARY STEEL DRILL PIPES  
Filed Nov. 12, 1947

2,641,488

FIG. 1.



FIG. 2.



*Inventors:*

JERRY JAY DUNN and  
WILLIAM O. CLINEDINST,  
by: *Donald G. Dalton*  
their Attorney.

## UNITED STATES PATENT OFFICE

2,641,488

METHOD AND MEANS FOR INCREASING  
BENDING FATIGUE STRENGTH OF RO-  
TARY STEEL DRILL PIPES

Jerry Jay Dunn, Ellwood City, and William O. Clineland, Pittsburgh, Pa., assignors to United States Steel Corporation, a corporation of New Jersey

Application November 12, 1947, Serial No. 785,432

3 Claims. (Cl. 285—146)

1

This invention relates to methods and means for increasing bending fatigue strength of rotary steel drill pipe.

Rotary drill pipe commonly comprises a number of steel pipe sections joined by interiorly screw threaded couplings that engage exteriorly threaded end regions of the sections. A frequent cause of failure in such pipe is through bending fatigue at the threaded joints, since the threads lower the bending fatigue strength of the pipe sections. Where such failure occurs, transverse fatigue cracks appear in the pipe section in the region of the last thread engaged by the coupling. Such cracks are produced by repeated bending of the pipe as it rotates within drill holes. Bending stresses are aggravated when the holes are not perfectly straight or when the drill string is partially in compression.

The stresses that cause fatigue failure in rotating drill pipe are distinctly different from those that cause fatigue failure in relatively fixed screw threaded fasteners. In the former fatigue failure is caused by repeated bending stresses, while in the latter fatigue failure is caused by repeated variations in longitudinal stresses. In view of this distinction the present application is confined to methods and means for increasing the bending fatigue strength of steel drill pipe.

An object of the present invention is to provide improved methods for increasing fatigue strength of steel drill pipe in regions of threaded joints, such methods involving cold working of the thread roots.

A further object of the invention is to provide methods for increasing fatigue strength of steel drill pipe threads beyond that obtainable through cold working conventional threads, the further increase being obtained by cutting the threads, and particularly the fade-out regions thereof, according to an improved design and subsequently cold working the roots.

A further object of the invention is to provide threaded steel drill pipe having improved means for restoring fatigue strength in the threaded region to approximately that of unthreaded pipe, such means including threads having cold worked root portions.

A further object of the invention is to provide externally threaded steel drill pipe having improved means for counteracting the loss in fatigue strength in threaded regions, such means including threads preferably of the V-type having roots rounded and cold worked at least from within the fade-out region to beyond the last

2

coupling-engaging thread, the sides and crests of the threads not being cold worked.

In accomplishing these and other objects of the present invention we have provided improved details of structure, preferred forms of which are shown in the accompanying drawing, wherein:

Figure 1 is a longitudinal sectional view through a portion of a drill pipe having threads cut and cold worked in accordance with the preferred embodiment of the present invention, and also illustrating the cold working tool in engagement with the threads; and

Figure 2 is a longitudinal sectional view through a portion of a drill pipe having threads cold worked in accordance with an alternative embodiment of the invention.

Referring more in detail to the drawing:

In Figure 1 there is shown a portion of a steel drill pipe 10 having a slightly tapered end. Exterior screw threads 11 are formed in said tapered end for engagement by a coupling, not shown. The threads may be either single or multiple and are preferably of the rounded V-type, having rounded roots 12, rounded crests 13 and sides 14. The threads have a fade-out region 15 extending into the body of the pipe section away from the coupling-engaging portion. In the preferred embodiment the thread roots in the fade-out region are also rounded and the fade-out angle, designated X, is as small as possible consistent with a relatively short fade-out region. Where possible, the fade-out angle is the same as the taper angle.

In accordance with the present invention, roots 12 of the coupling-engaging threads are cold worked as indicated at 16. Such cold working hardens the material at the thread roots and has been found to restore the fatigue strength of the threaded region to approximately that of unthreaded regions.

The roots are cold worked to a diameter reduction of at least 0.001". This lower limit is fairly critical since the cold working must first overcome the machining imperfections of the thread root and then provide a work hardening of the surface layer. While there are certain optimum upper limits for the cold working depending upon the steel grade, generally of the order of 0.003" to 0.004" diameter reduction of thread roots, increased amounts of cold working do not result in inferior product. If 0.006" diameter reduction is used on an API Grade D or E drill pipe steel, upsetting of thread flanks may occur unless restrained by the cold working tool or corrected for in the original thread pro-

file. Therefore, we wish to be restricted to an upper limit of cold work of not less than 0.008" diameter reduction, since satisfactory improvement in fatigue strength can be obtained by exceeding the optimum amount to at least this extent, although the operation is more difficult.

Only the thread roots are cold worked, since cold working makes the material hard and brittle and it is desired that the body of the threads be relatively soft for engagement with coupling threads and to prevent breakage.

Since fatigue failure almost invariably occurs in the region of the last thread on the pipe section engaged by the coupling, theoretically the increased fatigue strength could be obtained by cold working the root of only the last engaged thread. There are, however, practical difficulties to such practice, since it is not known in advance exactly which thread is to become the last engaged thread and since a continuous smooth thread root is desired. For these reasons, the preferred practice is to cold work the entire thread root, but to increase the amount of cold reduction progressively from the end of the pipe to a maximum within the diameter reduction range stated in the region which contains the last engaged thread, and then to decrease the reduction progressively through the fade-out thread.

In the preferred embodiment, shown in Figure 1, the rounded fade-out region of the thread is also cold worked. The alternative embodiment of the invention, shown in Figure 2, is similar to the embodiment shown in Figure 1, except that the threads in the fade-out region, designated 15a, are cut conventionally, and only the coupling engaging threads are cold worked. The fade out threads lack the rounded roots, and the fade-out angle, designated Y, is somewhat greater than in the preferred embodiment. Cold reduction of the thread roots of this alternative embodiment also provides increased fatigue strength over drill pipe in which the threads are not cold worked.

Cold working of external threads may conveniently be performed by rotating the pipe section against a tool such as that indicated at 17, Figure 1. Tool 17 includes a roller 18 having an edge 19 which fits within the pipe thread and contacts only the thread root. A hydraulic cylinder or other means, not shown, may be provided for applying sufficient pressure to the roller mounting for performing the cold work on the thread root. While the roller is illustrated as having but one root contacting edge, it is apparent that rolls having multiple edges likewise could be employed, and are preferred for cold working roots of multiple threads. Inasmuch as the tool and pipe rotating mechanism per se are not part of the present invention and a great variety of arrangements are obviously possible, no more detailed showing is deemed necessary.

Tests have demonstrated that the fatigue strength of drill pipe having threads cut and cold worked according to the preferred embodiment of the present invention is increased as much as 140% over that of pipes having conventional threads. The fatigue strength of drill pipe having threads cold worked according to the alternative embodiment is increased over that having conventional threads, but not to as great an extent as in the preferred embodiment.

As an example, comparative fatigue tests were conducted on 5 inch outside diameter, 0.362 inch

wall 18.50 lbs., threaded and coupled drill pipe of API Grade E steel. The pipe ends were upset to an outside diameter of 5.20 inches and an inside diameter of 3.750 inches and threaded with .200 inch pitch—.400 inch lead, rounded V-threads of API type. The threads in the fade-out region had the rounded roots preferred for cold working. The joint without cold worked roots had a satisfactory endurance limit or fatigue strength at a bending moment that creates a stress of 8,000 pounds per square inch maximum. Companion joints having the pipe thread roots cold worked according to the teachings of this invention resulted in fatigue strength of 19,000 pounds per square inch, representing an improvement of approximately 140%.

While rounded roots are preferable for accomplishing the maximum gain by cold working, it is possible to obtain considerable improvement in the fatigue strength thereby on flat and sharp roots. Modification of the V-thread, including the buttress, and acme types, may be so treated with benefit.

While we have shown and described only certain methods and means in which the present invention is involved, it is apparent that modifications may arise. Therefore, we do not wish to be limited by the disclosure set forth, but only by the scope of the appended claims.

30. We claim:

1. In a steel drill pipe section having external screw threads for engagement by an internally screw threaded coupling and having fade-out threads, the threads being of the V-type and having rounded roots, means for counteracting the loss of bending fatigue strength in the threaded region comprising cold worked portions in the roots of said coupling-engaging and fade-out threads, the amount of cold reduction progressively increasing from the end of the pipe section to the region of the last thread adapted to be engaged by the coupling and progressively decreasing through the fade-out threads.

2. In a steel drill pipe section having a tapered externally screw threaded end for engagement by an internally screw threaded coupling and having fade-out threads, the angle of fade-out being substantially equal to the angle of taper, the threads being of the V-type and having rounded roots, means for counteracting the loss of bending fatigue strength in the threaded region comprising cold worked portions in the roots of said coupling engaging and fade-out threads, the amount of cold reduction progressively increasing from the end of the pipe section to the region of the last thread adapted to be engaged by the coupling and progressively decreasing through the fade-out threads, the thread crests and sides being relatively soft.

3. A method for increasing bending fatigue strength of steel drill pipe sections at threaded regions which are adapted to engage a coupling comprising cutting in the end portions of the pipe external coupling-engaging and fade-out threads having rounded V-roots, and cold working the roots of both the coupling-engaging and fade-out threads throughout their length while maintaining the sides and crests of these threads in relatively soft condition, the degree of cold working gradually increasing from the thread at the end of the pipe to the region of the last coupling-engaging threads, where it produces a diameter reduction of 0.001 to 0.008 inch, and

gradually diminishing through the fade-out threads.

JERRY JAY DUNN.  
WILLIAM O. CLINEDINST.

| Number    | Name        | Date          |
|-----------|-------------|---------------|
| 2,243,608 | Schaurte    | May 27, 1941  |
| 2,261,056 | Dunn        | Oct. 28, 1941 |
| 2,284,260 | Castellanos | May 26, 1942  |

References Cited in the file of this patent

UNITED STATES PATENTS

| Number    | Name         | Date           |
|-----------|--------------|----------------|
| 631,158   | Echols       | Aug. 15, 1899  |
| 2,073,093 | Brantly      | Mar. 9, 1937   |
| 2,173,003 | Place        | Sept. 12, 1939 |
| 2,188,629 | Giese et al. | June 30, 1940  |

OTHER REFERENCES

Pages 96 through 98, Shot Peening, published in 1946 by American Wheelabrator & Equipment Corp., Mishawaka, Ind.

Arnold "Effect of Screw Threads On Fatigue," pages 497-505, Mechanical Engineering, July 1943, published by the American Society of Mechanical Engineers, New York, N.Y.